

## WATER-LAID FIBROUS SHEETS

Jay L. Piersol, East Hempfield Township, Lancaster County, Pa., assignor to Armstrong Cork Company, Lancaster, Pa., a corporation of Pennsylvania

No Drawing. Filed Nov. 12, 1957, Ser. No. 695,520

9 Claims. (Cl. 162—169)

This invention relates generally to water-laid fibrous sheets and more particularly to water-laid fibrous sheets having a synthetic rubber binder deposited on the individual fibers thereof. Still more particularly the invention relates to an improvement in the drainage rate of slurries wherein a synthetic rubber binder has been deposited on the individual fibers of the slurry by means of aluminum hydroxide.

A simplified flow diagram of the process is as follows:



In U.S. Patent 2,375,245—Pretzel, issued May 8, 1945, there is described a process of controlling the deposition of a synthetic rubber binder onto cellulosic fibers. The process contemplates pretreating the fibers with a water-soluble salt of aluminum, magnesium, or zinc, followed by the addition of ammonium hydroxide to form the insoluble metallic hydroxide. The subsequent addition of a synthetic rubber latex brings about the smooth and even deposition of the rubber particles on the individual fibers in the slurry. The rubber coated furnish fiber stock is then fed to a paper-forming machine such as a Fourdriner, cylinder machine, or the like. This process allows

2  
excellent control of the deposition of rubber on fibers in a papermaking slurry.

However, it has been found that aluminum hydroxide, because of its highly gelatinous nature, is a dispersing agent as well as a precipitating agent for rubber latices under the conditions described in the Pretzel process. The result of this situation is that a slow-draining stock sometimes results from use of the Pretzel process, particularly where higher amounts of aluminum hydroxide are formed in the slurry. Thus there is often a need for a modification of the Pretzel process which will produce a faster draining stock.

It is the primary object of the present invention to supply such a modification. It is a further object of the present invention to produce a papermaking furnish prepared by the Pretzel process which has a higher Canadian freeness than would normally be expected.

These objects are accomplished in a surprisingly straightforward and effective manner. The invention contemplates the addition of finely divided zinc oxide subsequent to the step of adding the ammonium hydroxide to form the metal hydroxide in the Pretzel process and prior to the step of adding the synthetic rubber latex. The result of the addition of zinc oxide at this point in the Pretzel process is that the stock possesses a higher Canadian freeness, presents a more clumpy appearance to the eye, and enables the formation of a thicker sheet.

The fibers contemplated for treatment by the present invention are cellulosic fibers such as kraft, rags, soda pulp, wood pulp, cotton linters, and the like. The fibers may be present in the slurry along with additional sheet-forming materials such as finely divided cork or finely divided scrap foam rubber; use of finely divided cork with fibers is fully described in U.S. Patent 2,613,190—Feigley.

35 The fibers and additional material, if any, are taken up in water in the usual manner to form a slurry which will generally be in the consistency range of about 0.5-5%. This slurry may then be subjected to mechanical refining in the usual refiners such as Jordan engines, beaters, disc refiners, and the like. When the desired degree of refinement has been achieved, the consistency may be adjusted to that desired for further treatment. Generally this consistency will be in the range of about 1-3%.

To the slurry there is then added a water-soluble salt 45 of a suitable electrolyte such as papermaker's alum, aluminum chloride, aluminum sulphate, magnesium chloride, magnesium sulphate, zinc chloride, and the like. For convenience the salt may be added in the form of its water solution. The amount of the electrolyte to be added will generally be in the range of about 25-75% by weight based on the amount of rubber to be deposited on the fibers subsequently.

After the electrolyte has been added to the slurry and dissolved therein, sufficient ammonium hydroxide is added 55 to establish a substantially neutral pH. To state it another way, sufficient ammonium hydroxide is added to react with and form the hydroxide of substantially all of the metal ion present in the aqueous phase of the slurry. The reaction proceeds rapidly, and gentle agitation for a few minutes is all that is needed.

Instead of adding next the synthetic rubber latex as contemplated by the Pretzel process, the present invention calls for the addition of zinc oxide at this point. The zinc oxide is preferably added in the form of a slurry in water; the slurry is simply poured into the papermaking slurry with gentle agitation. The zinc oxide is added as finely divided zinc oxide commonly known as pigment grade or filler grade zinc oxide; these are readily available in commerce. The amount of zinc oxide to be added will be controlled by the amount of aluminum hydroxide which has been formed in the papermaking slurry. Since the amount of aluminum hydroxide is controlled to some

extent by the amount of rubber to be deposited on the fibers, it can be seen that the amount of rubber ultimately controls the amount of zinc oxide to be added. Generally speaking, the zinc oxide will be added in an amount of about 3-50% by weight based on the total weight of rubber to be deposited on the fibers.

Upon the addition of zinc oxide to the papermaking slurry, some of the zinc oxide apparently immediately deposits on the aluminum hydroxide-treated fibers and some stays suspended in the water phase of the paper-making slurry. Once the zinc oxide has been thoroughly dispersed throughout the papermaking slurry, the synthetic rubber latex may be added.

The synthetic rubber latices contemplated for use in the present invention are those latices widely used in the beater saturation processes. Typical of these synthetic rubbers are the products known as GR-S, which is a copolymer of butadiene and styrene containing about 50% to about 70% butadiene. There may also be used those products known as Hycars, which are copolymers of butadiene and acrylonitrile containing about 50% to about 80% butadiene. The polychloroprenes may also be used. The polychloroprenes, often called neoprenes, are polymers of 2-chloro-butadiene-1,3. If desired homopolymers of butadiene may be employed as well as homopolymers and/or copolymers of butadiene homologues such as isoprene. These materials can be generally designated as synthetic rubbers and more specifically designated as rubberlike polymers of butadiene, isoprene, and chloroprene, and rubberlike copolymers of butadiene or isoprene with copolymerizable vinyl compounds such as styrene and acrylonitrile. As is well known in beater saturation methods, these synthetic rubbers are added to the slurry in the form of a latex. The rubber particles therein constitute an electronegatively charged organic binding material. These latices normally contain about 25% to about 50% by weight solids and contain additional compounding ingredients such as stabilizers and the like which are well known to the art and which form no part of this invention. The latices are added in an amount sufficient to introduce the required amount of rubber to be deposited on the fibers. Normally this will be in the range of about 10-100% by weight rubber based on the dry weight of the fibers.

The selected latex is simply poured into the zinc oxide treated slurry with gentle agitation. The rubber content of the latex coagulates and evenly deposits upon the fibers. Since zinc oxide is substantially insoluble in water under the beater saturation conditions of the Pretzel process, the rubber particles carry with them all the zinc oxide which is suspended in the white water. The resulting coated fibers carry an inner coating of zinc oxide and an outer coating of a synthetic rubber binder, which binder has distributed throughout additional particles of zinc oxide.

Agitation is maintained until rubber precipitation is complete. Normally the necessary period of time runs less than 20 minutes and often less than 10 minutes. Complete precipitation is indicated by the fact that the water phase of the papermaking slurry is water white and clear containing no suspended particles either of rubber or zinc oxide. The slurry itself will possess a more clumpy appearance to the eye than an identical slurry prepared without the use of zinc oxide. The Canadian freeness of the zinc oxide treated slurry will be higher than an identical slurry not treated with zinc oxide.

The specificity of zinc oxide as a means of improving drainage rate is unexpected and surprising. A series of similar compounds gives no improvement whatsoever. Zinc oxide appears to stand alone in this respect, the reasons for which are not understood.

The completed slurry is next formed into a sheet on the usual papermaking machine such as a Fourdrinier wire, cylinder machine, or the like. The resulting sheet on the wire, especially in heavier gauges, will be faster

draining due to the zinc oxide treatment. Sheets prepared according to the process of the present invention find use as a backing for linoleum composition and plastic surface coverings. Additionally, gaskets may be cut from the sheets, which gaskets find wide use in the automotive and airplane industries.

The following examples illustrate several embodiments of the invention. All parts are by weight unless otherwise stated.

#### Example 1

Into 3,750 parts of water there was placed 10 parts kraft fiber, and 20 parts of finely divided foam rubber scrap. There was then added 10 parts papermaker's alum dissolved in 100 parts of water, with gentle agitation. There was then added 8 parts ammonium hydroxide (28%) with continuing agitation.

A butadiene-styrene latex containing 50% styrene, 40% by weight solids (FRS-2000), was added to the resulting slurry in an amount of 45 parts. Antioxidants to stabilize the rubber against oxidation were also added, namely, 1.34 parts of a 45% dispersion of a mixture of mono- and di-heptyl diphenyl amines, and 0.75 part of polymerized 1,2-dihydro-2,2,4-trimethyl quinoline. Precipitation of the rubber was complete in 5 minutes.

A slurry identical to that described above was prepared save for the addition of zinc oxide subsequent to the addition of the ammonium hydroxide and prior to the addition of the synthetic rubber latex. The zinc oxide was added in the form of a 48% dispersion in water, and 1.56 parts of the dispersion was added.

The Canadian freeness of the stock containing no zinc oxide was 650 and the stock was only very slightly clumpy. The Canadian freeness of the stock containing the zinc oxide was 750 and the stock had a definite clumpy appearance to the eye.

Sheets were prepared from both stocks in a 12" x 12" laboratory mold and were subsequently dried in an air-circulating oven maintained at 195° F. The zinc oxide treated stock drained faster and allowed the production of a thicker sheet than did the stock not treated with zinc oxide.

#### Example 2

Two slurries were prepared having the ingredients listed below. The various ingredients were added in the order given.

|    | Ingredients                                                        | Run 1,<br>parts | Run 2,<br>parts |
|----|--------------------------------------------------------------------|-----------------|-----------------|
| 50 | Kraft Fibers.....                                                  | 7.5             | 7.5             |
|    | Cotton Linters.....                                                | 7.5             | 7.5             |
|    | Aluminum Sulphate.....                                             | 6.5             | 6.5             |
|    | NH <sub>4</sub> OH, 23%.....                                       | 5               | 5               |
|    | Zinc Oxide.....                                                    |                 | 1.58            |
| 40 | Butadiene-Styrene Copolymer Latex, 50%<br>Styrene, 40% Solids..... | 22.5            | 22.5            |
| 55 | Canadian Freeness.....                                             | 530             | 760             |

<sup>1</sup>(65% dispersion in water.)

The slurry prepared in run 1 was smooth while the slurry prepared in run 2 was very clumpy.

60 A run is prepared as in run 2 save that instead of butadiene-styrene copolymer latex there is added 22.5 parts of a butadiene-acrylonitrile copolymer latex containing 40% acrylonitrile (40% solids). The Canadian freeness of the resulting slurry is 750, while the Canadian freeness of an identical slurry prepared in the absence of zinc oxide is 510.

70 A series of runs was made as in run 2 except the following materials were used in lieu of zinc oxide: magnesium oxide, zinc sulphide, iron oxide (Fe<sub>2</sub>O<sub>3</sub>), chromium oxide (Cr<sub>2</sub>O<sub>3</sub>), and zinc sulphate. No change was noted in the drainage rate or clumpiness of the final slurry.

I claim:

1. In the process of producing felted fiber products by suspending fibers in a solution containing the dissolved

salt of the metal of the group consisting of aluminum, magnesium, and zinc, mixing with said solution and the fibers suspended therein an aqueous solution of ammonium hydroxide to a substantially neutral pH, and thereafter mixing with the thus treated fibers in suspension a latex of a synthetic rubber to form a papermaking slurry of rubber-coated fibers, the step of improving the drainage rate of said slurry by adding finely divided zinc oxide thereto subsequent to the addition of said ammonium hydroxide and prior to the addition of said synthetic rubber latex.

2. A process according to claim 1 wherein said zinc oxide is added in an amount of about 3-50% by weight based on the dry weight of said synthetic rubber.

3. A process according to claim 1 wherein said zinc oxide is added in the form of a dispersion.

4. A water-laid fibrous sheet comprising cellulosic fibers having an inner coating of zinc oxide and an outer coating of a synthetic rubber containing zinc oxide dispersed therethrough.

20

5. A sheet according to claim 4 containing zinc oxide in an amount of about 3-50% by weight based on the dry weight of said rubber.

6. A sheet according to claim 4 wherein said synthetic rubber comprises a butadiene-styrene copolymer.

7. A sheet according to claim 4 wherein said synthetic rubber comprises a butadiene-acrylonitrile copolymer.

8. A sheet according to claim 4 wherein said synthetic rubber comprises a polychloroprene.

9. A sheet according to claim 4 wherein said synthetic rubber is present in an amount of about 10-100% by weight based on the dry weight of said fibers.

References Cited in the file of this patent

UNITED STATES PATENTS

|           |                  |       |               |
|-----------|------------------|-------|---------------|
| 1,947,104 | Plumstead        | ----- | Feb. 13, 1934 |
| 2,375,245 | Pretzel          | ----- | May 8, 1945   |
| 2,666,699 | McQuiston et al. | ----- | Jan. 19, 1954 |
| 2,930,106 | Wrotnowski       | ----- | Mar. 29, 1960 |